

L. BREGUET.

CONNECTION OF TUBES OF DISSIMILAR METALS.

APPLICATION FILED NOV. 2, 1918.

1,347,075.

Patented July 20, 1920.

Fig.1.



Fig.2.



Fig.3.



Inventor:

Louis Breguet,

By Attorneys,

Drazen, Durk & Myers

# UNITED STATES PATENT OFFICE.

LOUIS BREGUET, OF VELIZY, FRANCE, ASSIGNOR TO SOCIETE ANONYME DES ATELIERS D'AVIATION LOUIS BREGUET, OF VELIZY, SEINE-ET-OISE, FRANCE.

## CONNECTION OF TUBES OF DISSIMILAR METALS.

1,347,075.

Specification of Letters Patent.

Patented July 20, 1920.

Application filed November 2, 1918. Serial No. 260,904.

To all whom it may concern:

Be it known that I, LOUIS BREGUET, a citizen of the Republic of France, residing in Velizy, Seine-et-Oise, France, have invented certain new and useful Improvements in the Connection of Tubes of Dissimilar Metals, of which the following is a specification.

This invention has for its object to provide very efficient connection of metal tubes and construction of tubular metal framework and the like, and is more especially intended for employment in joining tubes of aluminium, or of aluminium alloy, by means of steel connecting pieces and, in describing the invention we will presume that it is so employed.

In uniting such dissimilar metals by means of screwthreading, soldering or otherwise, there is encountered the difficulty that there is formed between the different metals an electrical couple which although very feeble, leads to the rapid disaggregation of the metals in intimate contact, and eventually destroys the connection, with the risk of causing serious accidents. Further, in the case of tubes of aluminum or aluminum alloys, which are produced by drawing, it is extremely difficult, or even impossible, to calibrate them to the exact diameter of the connecting pieces, so that there exists a play between the screwthreads and the connecting fittings.

To overcome these disadvantages, the present invention introduces the use as a solder or filling between the juxtaposed surfaces of the tube and junction piece, of sulfur applied in molten condition, so that it fills even the most minute spaces and serves not only to effect a firm mechanical engagement whereby looseness or play is avoided, but also serves as a dielectric to prevent electrolytic action between the dissimilar metals.

The following description with reference to the accompanying drawing of how the invention can be applied to the construction of the frame of the small boat of an airship will enable the nature of this invention and how it can be carried into effect to be understood.

Figure 1 represents the various members of the frame partly put together and Figs. 2, 3 and 4 show, respectively (drawn to a

larger scale) side, end, and plan views of one of the connecting pieces.

The tubes A, may be, for instance, of the aluminium alloy known as duralumin and circular in cross-section the outer surfaces of their extremities being roughened or striated, as shown at a.

The connecting pieces B may be of steel and these are roughened or striated on their inner surface as shown at b.

The tubes A, are engaged in the small tubular projections of the connecting-pieces B and are firmly fixed therein by means of sulfur brought to a liquid state by heat.

The great fluidity of molten sulfur allows it to fill up the smallest cavities which there may be in the roughened or striated surfaces and also to fill up any free space between the tubes A and the connecting-pieces B.

Although we have shown the tubes, and connecting-pieces B circular in cross-section, they may be of any other shape which may be desired.

This process allows of the employment, on a large scale, in aeronautical work, of the light aluminium alloy which is known as duralumin. This alloy may vary in composition according to the following percentages.

|                | H    | A    | B    | C    | D    | 85 |
|----------------|------|------|------|------|------|----|
| Copper.....    | 3.   | 3.5  | 4.2  | 4.9  | 5.6  |    |
| Manganese..... | 0.   | 0.5  | 0.6  | 0.7  | 0.8  |    |
| Magnesium..... | 0.5  | 0.5  | 0.5  | 0.5  | 0.5  |    |
| Aluminium..... | 96.5 | 95.5 | 94.7 | 93.9 | 93.1 | 90 |

What is claimed is:—

1. In a tubular structure comprising tubes and connecting pieces of dissimilar metals, the combination of a tube and connecting piece, the latter having a socket receiving the end of the former, and sulfur filling the space between their contiguous surfaces and serving as a dielectric to prevent electrolytic action.

2. In a tubular structure comprising tubes and connecting pieces of dissimilar metals, the combination of a tube striated at its end, with a connecting piece having a socket receiving such striated end, and sulfur filling the space between their contiguous surfaces.

3. In a tubular structure, the combination

of a tube of aluminium alloy, striated at its end, with a connecting piece of steel, receiving such striated end, and sulfur filling the space between their contiguous surfaces.

5. 4. In a tubular structure comprising tubes and connecting pieces having sockets for receiving the ends of the tubes, such

sockets making a loose fit with the tubes, the contiguous surfaces of the tubes and sockets being striated, and sulfur filling the space between such surfaces.

In witness whereof, I have hereunto signed my name.

LOUIS BREGUET.